# EUROPEAN PATENT SPECIFICATION

(11) **EP 0 018 335 B1**
(45) Date of publication and mention of the grant of the patent: **27.04.1983**
(21) Application number: 80850043.3
(22) Date of filing: 31.03.1980
(51) Int. Cl.: D03D 23/00

(54) **Cloth of high tensile and tearing strength**
Gewebe mit grosser Zugfestigkeit und grossem Reisswiderstand
Tissu à résistance élevée aux tensions et aux déchirures

(30) Priority: 02.04.1979 SE 7902880
(43) Date of publication of application: 29.10.1980
(73) Proprietor: ALMEDAHLS AB, S-510 50 Dalsjöfors (SE)
(72) Inventor: Ahlström, Sten, S-510 50 Dalsjöfors (SE); Zscherp, Rudolf, S-510 50 Dalsjöfors (SE)
(74) Representative: Wallin, John Erik

## Description

A cloth of high tensile and tearing strength is often used for technical purposes, such as tarpaulins, canopies, air-inflated structures and the like but also for many other products. Such a cloth comprises a ground fabric of multi-fibre, substantially equally coarse threads of polyamide, polyester or other synthetic material of high tensile strength, which are interwoven with the same set of warp and weft, the finished ground fabric being coated with a plastics or elastomer material, such as polyvinylchloride, polyurethane or a polymer of 2-chlorobutadiene. It is desired, with a given fabric weight per surface area, to obtain optimum strength properties of the coated fabric. To attain optimum strength properties it is essential to reach a balance of the tensile strengths in the warp and weft directions and at the same time a balance of the tearing strengths over warp and weft.

Generally, there is no problem in balancing the tensile strengths in the warp and weft directions. With the same yarn thickness for warp and weft said tensile strengths in fact are largely equally high, using the same set of warp and weft. Certainly, the weft mostly is slightly weaker but this difference is principally marginal and, if desired, can readily be balanced by a slight increase of the set of weft. It is considered that the somewhat lower tensile strength of the weft is due to the weft threads not lying quite as straight as the warp threads in the fabric. When being tested as well as in practical use the thread systems will therefore be placed under non-uniform load, resulting in a lower tensile strength in the weft direction.

A more complex problem is encountered with regard to the balancing of the tearing strengths over warp and weft. Starting from a plain cloth with 2 ends and fully symmetrical setting, the tearing strength over the weft will usually be only about 6096 of the value of the tearing strength over the warp. The explanation is that in the coating operation the coating material is urged in between the individual fibres in the weft yarn to a much greater extent than in the warp yarn. As a result, the weft yarn becomes stiffer and the tearing strength drastically decreases.

To compensate for this, one has in many cases turned to using a simple double-faced warp rib. It has thus been possible largely to triple the tearing strength over the weft, but at the same time the tearing strength over the warp decreased by about 20%, making the cloth still unbalanced.

Going the whole way and reinforcing the warp in the same manner, one will obtain a 2/2 dice weave. It has, however, been found that one must at the same time increase the set of both warp and weft by about 33% in order that the fabric shall permit being handled without any thread displacements. Now, the same thing happens again, i.e. the tearing strength over the warp triples whereas the tearing strength over the weft decreases by about 20%.

The object of the present invention is to eliminate the above-described problems encountered in providing balanced optimum strength properties in a cloth intended for technical purposes, such as tarpaulins, canopies, and the like, of the type indicated in the preamble of the appendant claim. This object has been realized in that the threads are interwoven in a weave pattern the repeat of which comprises six warp threads and six weft threads, the first and fourth weft threads passing over the first, second, fourth and fifth warp threads, the second weft thread passing over the first, third and sixth warp threads, the third weft thread passing over the second, third and sixth warp threads, the fifth weft thread passing over the third, fourth and sixth warp threads, and the sixth weft thread passing over the third, fifth and sixth warp threads.

The invention is based on the observation that it is possible, in connection with the plastics coating of ground fabrics, to attain balanced strength properties in the finished cloth by using for the manufacture of the ground fabric of the cloth a weave pattern that has been especially designed for the purpose. Said weave pattern is illustrated in the accompaning drawing. Each small square of the drawing corresponds to a point of cross-over of a warp thread and a weft thread, every horizontal row of squares thus corresponding to a weft thread and every vertical row of squares corresponding to a warp thread. The crossed squares indicate that the warp thread at the respective cross-over point passes over the weft thread while every empty square implies that the weft thread at the respective cross-over point passes over the warp thread. At the upper left of the drawing figure, thicker lines define a square comprising six warp threads and six weft threads. This is the pattern repeat for the weave pattern in question. The portion of the fabric pattern illustrated in the drawing comprises four pattern repeats for a clear showing of the nature of the pattern.

The repeat of the weave pattern illustrated in the drawing comprises, as mentioned above, six warp threads and six weft threads. The first and fourth weft threads pass over the first, second, fourth and fifth warp threads, the second weft thread passes over the first, third and sixth warp threads, the third weft thread passes over the second, third and sixth warp threads, the fifth weft thread passes over the third, fourth and sixth warp threads, and the sixth weft thread passes over the third, fifth and sixth warp threads.

Cloths having a ground fabric of the 2-end type, warp-rib type, 2/2 dice type and a ground fabric with a weave pattern according to the present invention were manufactured for illustration of the effect of the invention. The same yarn was employed for all ground fabrics, and the yarn was used for both the warp and the weft of the fabrics. The different ground fabrics were then coated with a plastics coat of the same kind and in the same manner, after which the finished cloths were subjected to tensile strength tests (5 cm wide strips) in both the warp and the weft direction as well as to tearing tests over both the warp and the weft. The results will appear from the following Table.

The Table shows that the cloth according to the invention had equally good and balanced tensile strengths in the warp and weft directions as the cloths having a weave with 2 ends and warp rib, but the tearing strengths over warp and weft were practically the same and substantially higher (approximately 100% or more) than the tearing strength in the poorest direction for the said two other cloths, simultaneously as the grammage and thickness of uncoated fabric and the set were practically the same in the three cases. With regard to the cloth having a ground fabric of 2/2 dice weave it should be observed that the tensile strengths and the tearing strength over the warp certainly were higher than for the cloth according to the invention, but the tearing strength over the weft was somewhat lower. Besides, it should be taken into consideration that the cloth of 2/2 dice weave, for the reasons earlier indicated, had to be woven with a substantially higher set and, consequently, substantially higher grammage and thickness for untreated fabric. Thus the cloth having a 2/2 dice weave was much more expensive to manufacture and had a substantially unbalanced tearing strength over warp and weft.

## Claims

Cloth of high tensile and tearing strength comprising a plastics- or elastomer-coated ground fabric of multi-fibre, substantially equally coarse threads which are interwoven with the same set of warp and weft, characterised in that the threads are interwoven in a weave pattern the repeat of which comprises six warp threads and six weft threads, the first and fourth weft threads passing over the first, second, fourth and fifth warp threads, the second weft thread passing over the first, third and sixth warp threads, the third weft thread passing over the second, third and sixth warp threads, the fifth weft thread passing over the third, fourth and sixth warp threads, and the sixth weft thread passing over the third, fifth and sixth warp threads.

## Revendications

Une étoffe à haute résistance à la traction et à la déchirure comportant un tissu fondamental enduit de matière plastique ou d'élastomère et constitué par des fils multifibre d'épaisseur sensiblement égale qui sont entrecroisés avec la même réduction de chaîne et de trame, caractérisée par le fait que les fils sont entrecroisés selon une armure dont le rapport comporte six fils de chaîne et six fils de trame, les premier et quatrième fils de trame passant par-dessus les premier, deuxième, quatrième et cinquième fils de chaîne, de deuixième fil de trame passant par-dessus les premier, troisième et sixième fils de chaîne, le troisième fil de trame passant par-dessus les deuxième, troisième et sixième fils de chaîne, le cinquième fil de trame passant par-dessus les troisième, quatrième et sixième fils de chaîne, et le sixième fil de trame passant par-dessus les troisième, cinquième et sixième fils de chaîne.

## Patentansprüche

Gwebe mit hoher Zugfestigkeit und hohem Reisswiderstand, umfassend eine mit Kunststoff oder Elastomer beschichtete Grundware aus mehrfaserigen, im wesentlichen gleich groben Fäden, die mit derselben Ketten- und Schussdichte verwebt sind, dadurch gekennzeichnet, dass die Fäden in einem Webmuster verwebt sind, dessen Bindungsrapport sechs Kettfäden und sechs Schussfäden umfasst, wobei der erste und der vierte Schussfaden über die ersten, zweiten, vierten und fünften Kettfäden verlaufen, der zweite Schussfaden über die ersten, dritten und sechsten Kettfäden verläuft, der dritte Schussfaden über die zweiten, dritten und sechsten Kettfäden verläuft, der fünfte Schussfaden über die dritten, vierten und sechsten Kettfäden verläuft, und der sechste Schussfaden über die dritten, fünften und sochsten Kettfäden verläuft.
